

# United States Patent Office.

---

LEVI S. ENOS, OF ALMOND, ASSIGNOR TO NATHANIEL SWEET, OF ALLEGANY COUNTY, NEW YORK.

*Letters Patent No. 77,874, dated May 12, 1868.*

---

## IMPROVED ALLOY FOR METALLIC ROOFING.

---

The Schedule referred to in these Letters Patent and making part of the same.

---

### TO ALL WHOM IT MAY CONCERN:

Be it known that I, LEVI S. ENOS, of Almond, in the county of Allegany, and in the State of New York, have invented certain new and useful Compounds for Metallic Roofing; and do hereby declare that the following is a full, clear, and exact description thereof.

The nature of my invention consists in the mixture of the following-named ingredients: Lead, (1) three-fourths of one pound; block-sin, one-fourth of one pound; antimony, (2) two drachms; and thereby making a compound, which I afterward roll out into sheets of any desired dimensions and thickness for roofing.

The compound, when made of the above ingredients, and rolled into sheets, makes a tenacious, pliable, and non-corrosive material, very desirable for roofing purposes, and may readily be applied to any roof, or be made to conform to any ordinary inequalities.

I do not wish to confine myself to any specific proportions of the above-named ingredients, as they may be varied so as to make the compound more rigid or pliable, as may be desired.

Having thus fully described my invention, what I claim as new, and desire to secure by Letters Patent, is—

The above-described compound, when made substantially in the manner and for the purpose specified.

In testimony that I claim the foregoing, I have hereunto set my hand, this 12 day of May, 1868.

LEVI S. ENOS.

Witnesses:

WESLEY BROWN,  
W. KNAPP.